

# United States Patent [19]

Katsitadze et al.

[11] 3,793,009

[45] Feb. 19, 1974

[54] **IMPACT ANTISPARK ALLOY FOR MACHINE PARTS**

[76] Inventors: **Shota Semenovich Katsitadze**, ulitsa Paliashvili, 102, kv. 4; **Dzhansug Illich Chkonia**, ulitsa Kipshidze, 5, kv. 24; **Alexandr Petrovich Martiashvili**, ulitsa Paliashvili, 82, kv. 6, all of Tbilisi, U.S.S.R.

[22] Filed: **Oct. 24, 1972**

[21] Appl. No.: **300,305**

[52] U.S. Cl. .... **75/159**, 75/153, 75/162

[51] Int. Cl. .... **C22c 9/06**

[58] Field of Search..... **75/153, 159, 162**

[56] **References Cited**

UNITED STATES PATENTS

|           |         |                       |          |
|-----------|---------|-----------------------|----------|
| 1,667,966 | 5/1928  | Corson.....           | 75/162   |
| 2,810,641 | 10/1957 | Roberts.....          | 75/162 X |
| 3,253,911 | 5/1966  | Cairns.....           | 75/159   |
| 3,297,497 | 1/1967  | Eichelman et al. .... | 75/162 X |

3,366,477 1/1968 Eichelman et al. .... 75/162 X

Primary Examiner—Charles N. Lovell  
Attorney, Agent, or Firm—John C. Holman

[57] **ABSTRACT**

A copper-based alloy also including aluminum and nickel and, additionally, chromium and zirconium, with all of the above components are taken in the following weight percent:

aluminum — 11.7-12.1

nickel — 7.5-8.2

chromium — 0.55-0.65

zirconium — 0.25-0.37

copper — the remainder

An advantage offered by the proposed alloy is that owing to the optimum composition of the alloy, said alloy possesses high physical and mechanical properties and is useful for manufacturing machine parts and tools noted for their strength, hardness and the absence of sparking.

**1 Claim, No Drawings**

## IMPACT ANTISPARK ALLOY FOR MACHINE PARTS

The invention relates to non-ferrous metallurgy and more particularly to alloys of precipitation hardening, which are used for manufacturing machine parts that do not cause sparking in mutual striking or upon striking other machine parts.

Copper-based alloys including aluminum amounting up to 10 weight percent and, up to 10 weight percent of various additives of which nickel may make up to 2 weight percent, iron — 4.5 weight percent, and manganese — 1.7 weight percent are known in the art (cf. French Pat. No. 1,176,757, cl. C22c, 1959).

As is known, the heat treatment of such alloys results in the separation of the dispersion particles of the intermetallides (Al Ni Fe), thus making said alloys stronger and harder.

A serious disadvantage of the known alloys is that they contain an explosion and risky element — iron, which markedly reduces the sphere of application of said alloys in the manufacturing of antisparking tools.

It is an object of the present invention to eliminate the abovementioned disadvantage.

Another object of the invention is to increase the strength and hardness of an alloy.

Another object of the invention is to obtain an optimum composition of the components providing high physical and mechanical properties for alloys and precluding sparking upon impact.

The element Zr also causes a reduction of the grain-size, which positively affects the strength of the alloy and reduces tendency to overheat at hardening temperatures.

5 The following is a detailed description and an exemplary embodiment of the proposed invention.

The proposed alloy contains in weight percent aluminum — 11.7-12.1; nickel — 7.5-8.2; chromium — 0.55-0.65; zirconium — 0.25-0.35, with copper constituting the rest of the alloy composition.

10 With the aluminum amounting to 12 weight percent, the alloy tends to become more brittle, and in order to increase the viscosity of said alloy, it is necessary to raise the nickel content to 8 percent.

15 With the increase in the nickel content makes the sphere of the brittle  $\gamma_2$  phase dependent upon a higher content of aluminum. That means that, with such percentage of aluminum, the separation of the  $\gamma_2$  phase occurs at a lower rate than is the case with a lower nickel content.

20 In nickel casting, the alloy offers the following indices for its physical and mechanical properties:

$$\sigma_{\beta} = 80-85 \text{ kg/mm}^2; \sigma_T = 65-68 \text{ kg/mm}^2; a_k = 2.5-3 \text{ kg/cm}^2;$$

$$\delta = 3-4 \text{ percent; and } H_B = 290-310.$$

The alloy thus produced was subjected to thermal treatment to secure higher strength.

25 The following is a table characterizing the mechanical indices of the proposed alloy:

| Mechanical indices<br>Variations of thermal treatment                                                     | $\text{kg/mm}^2$<br>$\sigma_{\beta}$ | $\text{kg/mm}^2$<br>$\sigma_T$ | $\text{kgm/cm}^2$<br>$A_k$ | %<br>$\delta$ | $H_B$   |
|-----------------------------------------------------------------------------------------------------------|--------------------------------------|--------------------------------|----------------------------|---------------|---------|
| Heating to 950-970°C, soaking for 1-1.5 hour, water hardening; tempering to 530-550°, soaking for 4 hours | 95-100                               | 78-83                          | 2-2.2                      | 2.5-3         | 320-330 |
| Heating to 920-940°, soaking for 1 hour, water hardening; tempering to 490-510°, soaking for 2 hours      | 85-90                                | 75-78                          | 1-1.5                      | 2-2.5         | 340-360 |
| Heating to 880-900°, soaking for 30-35 min, water hardening; tempering to 450-470° soaking for 35-40 min. | 80-85                                | 73-77                          | 0.8-1                      | 1-1.5         | 370-390 |

45

These and other objects of the present invention have been achieved by providing an alloy for manufacturing machine parts that does not cause sparking upon impact, and which is based on copper but also includes aluminum and nickel, with said alloy additionally containing, according to the invention, chromium and zirconium, with all of the abovementioned components taken in the following weight percentage:

aluminum — 11.7-12.1

nickel — 7.5-8.2

chromium — 0.55-0.65

zirconium — 0.25-0.35

copper — the remainder

By including such elements as chromium and zirconium into the alloy, it is possible to ensure the separation of intermetallide  $\text{Cr}_2\text{Zr}$  in the course of thermal treatment. Also separated in the form of a dispersion in said alloy is an intermetallide of NiAl. The combined separation of these two intermetallides helps to secure the high physical and mechanical properties of the alloy.

In thermal treatment according to the first variation, a separation of the  $\text{NiAl}$  and  $\text{NiAl}_3$  phases are observed, as well as the  $\text{Cr}_2\text{Zr}_2$ .

50 In thermal treatment according to the second variation, in addition to the above phases, a partial disintegration of phase  $\beta$  into  $\alpha + \gamma$  is observed. As phase  $\gamma$  is superhard, the effect of the alloy hardness increase was obvious.

55 Thermal treatment according to the third variation ensures a complete disintegration of phase  $\alpha\beta$  into  $\alpha + \gamma$ .

The proposed alloy is characterized by a high ratio  $\sigma_T/\sigma_B$  ratio both in the as-cast and, particularly, the thermally treated state.

60 Both the as-cast alloy and the thermally treated alloy do not cause sparking even in the case of an impact against a steel plate with a force of 145 kGm.

65 Adequately high mechanical properties ( $\sigma_{\beta}$ ,  $\sigma_T$  and  $H_B$ ) of the proposed alloy make it quite useful in machine building for manufacturing machine parts and for tools standing out for their strength, hardness and the absence of sparking.

What we claim is:

1. An alloy for manufacturing machine parts that do not cause sparking upon impact, said alloy comprising the following components taken in weight percent:

aluminum — 11.7-12.1

nickel — 7.5-8.2  
chromium — 0.55-0.65  
zirconium — 0.25-0.35  
copper — the remainder to 100 percent.

\* \* \* \* \*